

## UNITED STATES PATENT OFFICE

2,193,241

## POLISH

Martin J. Seuberling, Cincinnati, Ohio, assignor, by mesne assignments, to Vegetable Oils Specialty Corporation, Cincinnati, Ohio, a corporation of Ohio

No Drawing. Application August 23, 1935,  
Serial No. 37,508

4 Claims. (Cl. 134—24)

This invention relates to a liquid polish of the emulsion type for brightening the appearance of finished wood, metal and like surfaces, and also relates to a method of making the same.

5 More particularly, the invention relates to a liquid polish embodying the virtues in finishing of so-called "French polish," but not attended by the great difficulties of application which characterize the latter.

10 "French polish," as the term is used, refers to the old-fashioned method of polishing surfaces, especially wood, by vigorously and strenuously applying a mixture of shellac and oil with a rag, and continuing rubbing with the rag until the shellac becomes dry and the surface presents a 15 lustrous and somewhat burnished appearance.

The term "French polish" is almost synonymous with hard work. This invention discloses a 20 means for obtaining a polish of such characteristics without the necessity of vigorous rubbing or burnishing.

It is therefore an object of the invention to provide a polish which is cheap to make but very effective to use for polishing wood or metal, varnish or lacquered surfaces.

25 A polish manufactured from a shellac and oil base while difficult to obtain, presents after its application, a surface of very superior qualities. In the first instance, the polish film is of a harder 30 nature and not susceptible to the usual marring characterizing so-called wax or wax emulsion polishes. Secondly, the surface so prepared is not comprised of oxidizable substances and hence retains its lustre without dulling for an appreciably longer period than does the wax or wax 35 emulsion type of polish. In another aspect the resultant shellac and oil film obtained is free from the disadvantage of water or rain spotting. These characteristics make the composition disclosed herein admirably adapted to use in the 40 polishing of automobiles and the like.

Briefly, the invention disclosed herein comprises a liquid polish responsive to these objects, and which is superior to the substances heretofore 45 available in that it does a better job of relusterizing the original finish of a given wood or metal surface, in that it requires no preferred procedure in use to obtain best results, in that it does not water spot, and in that it may be applied to the 50 whole of a given surface to be treated, e. g., an automobile or piece of furniture, and thereafter the whole surface subsequently wiped off and lusterized as distinguished from the conventional way and necessity of treating and then polishing subdivided increments of the whole of a given 55 surface.

To achieve the resultant qualities of a French 60 polish, while circumventing the objectionable necessity of vigorousness in the polishing operation, constitutes an appreciable problem. A

shellac and oil mixture is thick and heavy and difficult to use correctly. The conventional solvents for shellac are likewise the conventional solvents for most types of finishes and therefore an attempt to reduce the viscosity of the liquid 5 by such materials is dangerous. Both shellac and oil are incompatible with water. Hence, water, as a diluent, if associated with the other components in a conventional emulsifying manner, is not satisfactory because of the rapidity of 10 separation, and failure of consistency and results. Furthermore, attempts to emulsify the shellac and oil in the water in the conventional manner are likewise unsatisfactory.

I have devised a composition which includes 15 in its ingredients shellac, oil, water, and an abrasive wherein the components are so related that the foregoing objectives in polishing are readily accomplished by first associating the shellac and oil with the abrasive particles as a 20 film coating therefor, and then wetting and dispersing in aqueous solution the discrete particles so enfilmed. The method aspect of the invention resides in the means by which the composition is effected.

The preferred ingredients of my composition 25 are liquid shellac, mineral oil, an abrasive such as diatomaceous earth or tripoli, water, glycerine, and a dispersion stabilizer, or interfacial tension depressant such as soybean phosphatides dissolved in a small quantity of alcohol or other 30 suitable solvent. The mineral seal oil is preferably of a viscosity heavier than kerosene but completely volatile. The mineral seal oil and the shellac are associated with the abrasive 35 particles as film-like coatings. These in turn are rendered wettable by the water and glycerine solution through the interfacial tension depressing action of the soybean phosphatides, the latter substance in turn further assisting in maintaining the dispersed particles in appropriate 40 relation throughout the mass of liquid so constituted.

A preferred formula is set forth below by way 45 of example.

Formula for 4½ gallons:

|                                        | Pounds |
|----------------------------------------|--------|
| Shellac (orange-white)                 | 1 ¾    |
| Alcohol and 2 oz. soybean phosphatides | ¼      |
| Mineral seal oil                       | 8 ¾ 50 |
| Diatomaceous earth                     | 5 ½    |
| Water                                  | 17     |
| Glycerine                              | ¾      |

A diatomaceous earth may be of the filter cell 55 grade or, if a less vigorous abrasive or cleaning agent is desired, air floated diatomaceous earth may be used. Equally suited to use and of slightly better cleaning action than diatomaceous earth alone is a mixture of air floated diatomaceous 60

earth and twice ground rose tripoli, these preferably being in equal parts by weight. The shellac may be of the orange or white grade. The chemical lecithin or other suitable dispersing agents 5 may be used in place of the soybean phosphatides disclosed above. The glycerine in the composition prevents the abrasive from becoming dust-like after the polish has dried, and thus from contaminating the finished surface after final polishing.

10 The method aspect of the invention resides in the process by means of which the abrasive or cleaning agent is enfilmed with shellac and mineral oil. This process comprises first placing 15 the appropriate amounts of shellac and mineral oil into a tank and mixing them together until the mixture is of uniform consistency and thereafter or simultaneously adding to this mixture the soybean phosphatides in a suitable solvent 20 such as alcohol. To the mixture so constituted is added and mixed the desired quantity of cleaning powder or abrasive. Upon mixing the mass becomes of a thick and plastic consistency, not unlike the consistency of dough or wood putty. In 25 this operation the particles of the abrasive are wetted and entrained within the "French" polish component of the composition. Finally, water in the desired quantity is added to reduce the consistency of the mixture to an appropriately liquid state.

30 From sixteen to twenty-five pounds of water, using the indicated percentages in the example listed heretofore, may be used without dispelling shellac from the mixture. A slight precipitation 35 occurs if a larger quantity of water is used, and this precipitate is similar in appearance to small chunks of wood. As an aid to suspension a small quantity of bentonite may be used. From about one-half percent to about two percent is very 40 effective.

45 Too great deviation in the sequence steps of the process disclosed above should be avoided because the components of the polish are inherently incompatible and their proper assimilation is otherwise quite difficult.

50 The polish prepared according to the disclosure herein is applied to the surface in the conventional manner with a soft rag and with a gentle rubbing motion. During this period the abrasive removes any dirt film or the like and after removal, there is disposed upon the surface thus easily wetted a thin but adequate film of French polish.

In this operation divisional portions of the whole surface need not be separately treated, but rather the entire surface to be polished can be gone over during the application step, and thereafter gone over in the final polishing step. In this polishing operation the surface so treated is preferably wiped with a clean rag in several passes, after which the surface is left in a brilliant and pleasing condition.

5 Having described my invention, I claim: 10

1. A wood and metal polish, which comprises, abrasive particles enfilmed with a coating of shellac and mineral oil, said particles dispersed in water solution by the aid of an interfacial tension depressant, the composition by virtue of the 15 relationship possessing the capacity to apply shellac evenly and uniformly to a surface as the abrasive removes dirt film from the surface.

2. As a new product, a polish for wood and metal surfaces, which polish comprises, abrasive 20 particles, carrying in film-like manner a coating of shellac and mineral seal oil, said abrasive containing soybean phosphatides, the said product when applied with a rag, possessing the capacity to provide the film of shellac on a surface as the 25 abrasive removes dirt from the surface homogeneously dispersed in aqueous solution.

3. As a new product, a polish for wood and metal surfaces, containing shellac, mineral oil, finely divided particles of abrasive and water, in 30 which composition approximately one and three-fourths parts of shellac and approximately eight and three-fourths parts of oil are carried by approximately five and one-half parts of abrasive, and the particles of abrasive carrying the shellac 35 and oil homogeneously are dispersed in the water, the shellac and the oil components forming a film coating for the particles of abrasive.

4. As a new product, a polish for wood and metal surfaces, containing shellac, mineral oil, 40 finely divided particles of abrasive and water, in which composition approximately one and three-fourths parts of shellac and approximately eight and three-fourths parts of oil are carried by approximately five and one-half parts of abrasive 45 and the particles of abrasive carrying the shellac and oil homogeneously are dispersed in the water in the presence of soybean phosphatides, the said shellac and oil components forming a film coating upon the surface of the particles of abrasive. 50

MARTIN J. SEUBERLING.